

# UNITED STATES PATENT OFFICE.

RUSSELL WILLIAM MUMFORD, OF NEW YORK, N. Y., ASSIGNOR TO REFINING PRODUCTS CORPORATION, OF WILMINGTON, DELAWARE, A CORPORATION OF DELAWARE.

## PROCESS OF MAKING DECOLORIZING CARBONS.

1,359,094.

Specification of Letters Patent. Patented Nov. 16, 1920.

No Drawing.

Application filed March 23, 1918. Serial No. 224,199.

To all whom it may concern:

Be it known that I, RUSSELL WILLIAM MUMFORD, a citizen of the United States, residing at New York, in the county of 5 New York and State of New York, have invented certain new and useful Improvements in Processes of making Decolorizing Carbons, of which the following is a specification.

10 This invention relates to processes of making decolorizing carbons; and it comprises a method, of making decolorizing carbon wherein finely powdered coal, lignite or brown coal is admixed with various 15 agents, such as milk of lime and phosphate solution, ammoniacal tar, etc. together with, usually, a mineral spacing agent, such as dolomite, and is gradually heated through a wide range of temperatures extending 20 above 600° C.; all as more fully hereinafter set forth and as claimed.

“Decolorizing carbon” is the commercial name now given to certain carbon preparations made from vegetable materials and 25 distinguished from charcoal and the like, by a high power of decolorizing liquids such as sugar solutions. These decolorizing carbons are even more active in their absorbing and decolorizing power than is 30 boneblack and can be used for many purposes for which boneblack is not suitable. For the most part, they occur as very fine powders; a very finely pulverulent state being considered necessary to give a large area 35 of surface; the large surface upon which their high degree of activity, at least in part, depends. While they are efficient in removing color from sugar solutions, oils and the like, they are not active in removing 40 fine suspended solids; and they do not give “bright” or clear solutions. In fact, because of their fineness, they often rather contribute to the turbidity, some portion of the carbon remaining in suspension and forming 45 a blackish cloud. In the use of decolorizing carbons it is therefore common to follow them with a clarifying agent having the power of removing suspended solids, such as kieselguhr. In another application, Serial 50 No. 167,971 filed May 11, 1917, (Patent No. 1,286,187, Nov. 26, 1918,) I have described and claimed a method of making decolorizing carbons which not only have a high activity as regards decolorization but are

also active in removing suspended solids; 55 that is they not only have a decolorizing action but also a clarifying action. Briefly stated, this method comprises making a mixture of a vegetable material, such as sawdust or peat, with various colloids 60 and charring the mixture slowly through a range of temperatures ending above 600° C. In charring any vegetable matter the first effect is the production of various tars, gases, vapors, etc. These products in their turn carbonize with the separation of more carbon. The carbon coming directly from the vegetable material may be called primary carbon and that formed by heating the volatile products may be called 65 secondary carbon. With any quick heating action the secondary carbon tends to form in the pores of the primary carbon and clog them. This is very undesirable. By the slow heating in the invention of said prior 70 application I afford time for the volatile products to escape from the pores of the primary carbon, thereby securing an unclogged, highly effective material. In order to aid in securing this result, I ordinarily 75 space apart the particles of the vegetable matter with a mineral powder of some character. I may use a calcareous material known as dolomite which is a magnesian limestone or mixture of carbonates of magnesia and lime and which evolves carbon dioxid at relatively low temperatures, beginning at 250° C. The magnesium carbonate first loses CO<sub>2</sub> and then the calcium carbonate, so there is a slow and continuous 80 evolution of carbon dioxid throughout the operation. This carbon dioxid not only serves to sweep away the primary vapors of charring but it is itself adsorbed in the char to a greater or less extent and as the temperature goes up it has a chemical and probably also mechanical influence on the carbon. It tends to keep the pores free and to clean, and probably, to some extent at least, to widen them somewhat. After the 85 char is complete the mineral matter may be removed in various ways.

I explained in Patent No. 1,286,187 that as a rule I found it better not to have the raw material from which the carbon is 90 made too solid or compact in structure, and that I usually preferred to use materials which are porous enough to have the

power of absorbing water in a substantial amount. I have found, however, that a very efficient type of decolorizing carbon can be made of carboniferous materials of 5 more or less compact structure such as lignite, brown coal, or any other coal or coaly material high in volatile matter, by mixing them in a powdered condition with a tarry liquid or tarry matters, such as the 10 residues of tar distillation (pitch) to which advantageously ammoniacal liquor may be added. I have found that if I mix coal, brown coal or lignite, which should be reduced to a fine powder of, say, 80 to 150 15 mesh, with ammoniacal tar, such as is produced in gas works, and then char I obtain a material which is highly efficient as a decolorizing and clarifying agent. The crude tar from the gas works, which always 20 contains more or less ammonia, may be used; or tarry ammonia water may be employed. In either event the coal or lignite powder is made into a dough-like mass with the tar or tarry water, formed into 25 pellets or the like, and heated slowly through a range of temperatures ending above 600° C. In some cases I may mix the powdered brown coal with milk of lime or a mixture of milk of lime and solution 30 of monocalcium phosphate and char in the same way; but in the present invention I prefer the use of ammoniacal tar. Ammoniacal tar may also be used in connection with the other materials. A useful 35 mixture may be made as a dough-like composition of powdered coaly matter and ammoniacal tarry matter with a watery solution of milk of lime and monocalcium phosphate. A certain proportion of mineral 40 spacing agent, which is advantageously dolomite, may be mixed in with the other materials prior to forming the dough. Other tarry materials than gas tar such as the residues of tar distillation and similar 45 products, or such as asphaltic materials, may be mixed with the coal, but I find ammoniacal tar to be the best material.

The charring may be performed in any suitable type of venter retort by any suitable 50 method of heating. In order to sweep out the volatile products formed in charring, currents of steam or products of combustion may be blown through the retort. In one advantageous method of charring 55 which I sometimes employ, (see my Patent No. 1,287,592) I may place the mass to be charred in shallow covered trays and pass them through a tubular tunnel-like chamber heated by what is known as "surface 60 combustion" therein. In surface combustion, as the term is understood today, the exact quantities of air and gas are used together, and burnt in the pores of refractory material. In so doing there is no excess of oxygen in the products of combustion.

tion to waste away the material to be charred.

After the carbon is produced it may be cooled by continuing the blowing through 70 of steam or it may be moistened at once to cool it rapidly and prevent spontaneous ignition and then the mineral matter, if such be used, may be removed by sedimentation and acids if desired. The carbon is then dried. I find it advantageous to 75 perform the drying in a rotary tube by the waste gases from the firing means used in charring.

In a specific embodiment of the present invention I take brown coal of any suitable 80 kind and grind it to about 80 mesh. The comminuted brown coal I mix with about 5 to 30 per cent. of finely powdered dolomite and convert the mixture into a dough-like plastic mass with wet ammoniacal gas 85 tar, using the amount of tar which may be necessary to give the desired consistency. The mass is next formed into pellets and placed in a vented retort. A current of dry steam is passed through the retort and the 90 heat is slowly raised until it finally reaches 600° C. or higher. Finishing at a very high temperature is necessary in order to insure as far as practicable the charring of anything soluble in the material. In the final 95 product there must be no uncharred material.

After the charring is finished steam is allowed to continue to pass through the retort to cool the material until it is sufficiently cool to be exposed to the atmosphere 100 without danger of ignition.

In using ammoniacal tarry materials with the coal, the resulting product is a mixture of two kinds of carbon, one coming from 105 the coal and the other from the tarry materials. The resultant product also contains more nitrogen than would the coal charred alone. The condition or form of combination in which this nitrogen exists is not 110 known. For some reason the presence of this nitrogen in the product is advantageous to its decolorizing properties.

What I claim is:

1. The process of making a decolorizing 115 carbon which comprises comminuting coaly matter high in volatile constituents, mixing with tar and ammonia and charring through a range of temperatures slowly rising to above 600° C.

2. The process of producing decolorizing carbon which comprises making a doughlike mixture of powdered coaly matter with tarry matter and ammonia and charring the same in a vented retort through which a 120 draft current of dry steam is passed to facilitate removal of vapors and continuing the heating through a range of temperatures slowly rising above 600° C.

3. The process of producing decolorizing 130

carbon which comprises making a doughlike mixture of powdered coaly matter with ammoniacal tarry liquid from gas works and charring the same in a vented retort 5 through which a draft current of dry steam is passed to facilitate the removal of vapors and continuing the heating through a range of temperatures slowly rising above 600° C.

4. The process of producing decolorizing 10 carbon which comprises making a doughlike mixture of powdered coaly matter and the residues of tar distillation with ammoniacal liquor, and charring the same in a vented retort through which a draft current of dry 15 steam is passed to facilitate the removal of vapors and continuing the heating through a range of temperatures slowly rising above 600° C.

5. The process of producing decolorizing 20 carbon which comprises making a doughlike mixture of powdered coaly matter and tarry matter with ammoniacal liquor and charring the same in a vented retort through which a current of dry steam is passed to 25 facilitate removal of vapors, and continuing the heating through a range of temperatures slowly rising above 600° C.

6. The process of producing decolorizing carbon which comprises comminuting coaly matter high in volatile constituents, mixing 30 with tar and ammonia and a mineral powder and charring through a range of temperatures slowly rising to above 600° C.

7. The process of producing decolorizing carbon which comprises making a mixture 35 of powdered coaly matter and tarry matter containing ammonia with calcareous matter and charring same through a range of temperatures slowly rising to above 600° C.

8. The process of producing decolorizing 40 carbon which comprises making a doughlike mixture of powdered coaly matter and ammoniacal tarry matter with a watery solution of milk of lime and monocalcium phosphate, charring the mixture in a vented re- 45 tort, through which a current of dry steam is passed to facilitate removal of vapors, continuing the heating through a range of temperatures slowly rising above 600° C., and cooling the finished product by passing 50 a current of steam through the retort.

In testimony whereof I affix my signature hereto.

RUSSELL WILLIAM MUMFORD.